

1

3,377,219

## NITRATED ORGANIC LIQUID PROPELLANT COMPOSITION HAVING IMPROVED SPARK IGNITION

Ludwig Stiefel, Philadelphia, and Howard A. Kirshner, Levittown, Pa., assignors to the United States of America as represented by the Secretary of the Army  
No Drawing. Filed Sept. 28, 1964, Ser. No. 399,943  
4 Claims. (Cl. 149—88)

### ABSTRACT OF THE DISCLOSURE

Liquid propellants capable of ready ignition by a submerged spark therewithin, the spark requiring but little energy to cause its formation due to the composition of said propellant which includes either a quaternary ammonium salt or colloidal graphite.

The invention described herein may be manufactured and used by or for the Government for governmental purposes without the payment to us of any royalty thereon.

This invention relates to spark ignition of liquid propellants and particularly, to submerged spark ignition of non-conductive organic liquids used as propellants.

Many organic liquids including nitromethane, nitropropane, alkyl nitrates, and nitrate ester compounds are commonly employed as liquid propellants. Certain applications of these propellants require that they be ignited by electrical spark discharge generated across electrodes submerged in the propellants. However, efforts to conveniently ignite the propellants by this electrical spark discharge method have resulted in virtual failure. At the root of the problem is the very high order of electrical energy required for generating the ignition spark. The size and extent of the equipment necessary to provide this energy has been such as to render the method impractical. A principal reason advanced for the high electrical energy required for spark ignition is the poor electrical conduction properties of the propellants.

It is, therefore, an object of this invention to provide organic liquid propellants characterized by improved electrical conduction properties.

A further object is to provide a method for enhancing the electrical properties of organic liquid propellants to permit practical submerged spark ignition thereof.

The above and other objects are attained by adding into organic liquid propellants or blends thereof small amounts of either low molecular weight quaternary ammonium salts or colloidal graphite. For example, igniting

rate propellant having increased electrical conductivity characteristics is obtained. Accordingly, the electrical energy required to generate the ignition spark is considerably diminished.

The improved propellants of this invention comprise any non-conductive, organic liquid propellants to which have been added between 0.5% and 3.0% by weight of an additive selected from the group consisting of a quaternary ammonium salt and colloidal graphite. In the case of the former, dissolution occurs in the propellant while in the case of the latter the graphite remains in suspension. However, the results in any of the above mixtures are the same, that is, in comparison with non-conductive, organic liquid propellants not having the additives mentioned, substantially lower electrical energies are necessary for generating ignition sparks across electrodes submerged in the propellants.

The following examples further illustrate the invention, which is not to be construed as limited thereby. Various quaternary ammonium salts as well as colloidal graphite were mixed under ambient conditions with base propellants. The examples are shown in the following table.

| Ex. No. | Base Propellant                        | Additive and Quantity Thereof                   |
|---------|----------------------------------------|-------------------------------------------------|
| 1       | 60% Ethyl Nitrate, 40% Propyl Nitrate. | 1.5% by weight colloidal graphite.              |
| 2       | 60% Ethyl Nitrate, 40% Propyl Nitrate. | 1.5% by weight tetra ethyl ammonium chloride.   |
| 3       | 60% Ethyl Nitrate, 40% Propyl Nitrate. | 0.5% by weight tetra n-propyl ammonium nitrate. |
| 4       | 100% Propyl Nitrate.                   | 3.0% by weight tetra n-propyl ammonium nitrate. |

To illustrate the improved spark ignition characteristics of the propellants of this invention, spherical tipped stainless steel electrodes having a  $\frac{1}{16}$  inch diameter were submerged into an open cup of propellants of compositions set forth in the above examples. Two sets of electrodes having spark gaps of 0.042 and 0.050 inch respectively were used, both being connected to a 5000 volt, 6.0 microfarad variable capacitance electrical system. Electrical energy was applied until a spark was generated across the electrodes and the propellant ignited. The total energy required for ignition of the propellants was computed from the formula,  $W = \frac{1}{2}CV^2$  where  $W$  is total energy in joules,  $C$  is capacitance in farads, and  $V$  is voltage applied in volts. The above procedure was applied to testing propellants without the additive of this invention. Results of the foregoing tests are given in the following table.

TABLE II.—EFFECT OF ADDITIVES UPON SPARK IGNITION ENERGY

| Example No. | Composition                                                                                                   | Electrode Gap, inches | Voltage Applied, volts | System Capacitance, microfarads | Energy Applied, joules | Results      |
|-------------|---------------------------------------------------------------------------------------------------------------|-----------------------|------------------------|---------------------------------|------------------------|--------------|
| 1.          | Base propellant: 60% Ethyl Nitrate, 40% Propyl Nitrate, no additive.                                          | 0.042                 | 5,000                  | 6.0                             | 75                     | No ignition. |
| 2.          | Base propellant: 60% Ethyl Nitrate, 40% Propyl Nitrate, 1.5% by weight colloidal graphite added.              | 0.042                 | 2,100                  | 4.0                             | 8.8                    | Ignition.    |
| 3.          | Base propellant: 60% Ethyl Nitrate, 40% Propyl Nitrate, 1.5% by weight tetra ethyl ammonium chloride added.   | 0.042                 | 2,100                  | 3.0                             | 6.6                    | Do.          |
| 4.          | Base propellant: 60% Ethyl Nitrate, 40% Propyl Nitrate, 0.5% by weight tetra n-propyl ammonium nitrate added. | 0.050                 | 3,000                  | 1.0                             | 4.5                    | Do.          |
|             | Base propellant: 60% Ethyl Nitrate, 40% Propyl Nitrate, no additive.                                          | 0.050                 | 5,000                  | 1.0                             | 13                     | No ignition. |
|             | Base propellant: 100% propyl nitrate, 3.0% by weight of tetra n-propyl ammonium nitrate added.                | 0.050                 | 2,700                  | 2.0                             | 7.0                    | Ignition.    |
|             | Base propellant: 100% propyl nitrate, no additive.                                                            | 0.050                 | 5,000                  | 6.0                             | 75                     | No ignition. |

an ethyl-propyl nitrate propellant without these additives by means of a spark generated between electrodes submerged in the propellant requires a relatively high electrical energy. This is attributed to the low electrical conductivity of the propellant. By adding a quaternary ammonium salt or colloidal graphite, an ethyl-propyl ni-

70 The data in the foregoing table demonstrate the significant improvement in spark ignition of non-conductive, organic liquid propellants as a result of the addition thereto of quaternary ammonium salts or colloidal graphite. The data show that with the inventive additives the energy required to generate an ignition spark is decreased by a

factor of as high as 15. This figure is conservative since the electrical system used did not have the capacity to demonstrate the ignition of the base propellants tested without additives.

Various other quaternary ammonium salts were added to different organic liquid propellants and tested for spark ignition energy. The aforementioned procedure was followed in all cases. The test results were favorable in that ignition was achieved at an energy level well below that necessary for ignition of propellants without the additives of this invention. The following are illustrative of such other quaternary ammonium salts tested:

Tetramethyl ammonium bromide  
 Tetraethyl ammonium bromide  
 Tetraethyl ammonium chloride  
 Tetra-n-propyl ammonium nitrate  
 Tetra-n-propyl ammonium iodide  
 Tetra-n-butyl ammonium iodide  
 Tetra-n-butyl ammonium picrate

Since many examples of the foregoing compositions may be made without departing from the scope of the invention, the foregoing is to be interpreted as illustrative only, and not as defining or limiting the scope of the invention.

We claim:

1. An improved liquid propellant consisting essentially of an electrically non-conductive, nitrated organic liquid propellant and an additive selected from the group consisting of quaternary ammonium salts and colloidal graphite, said additive being present in an amount effective to permit practical spark ignition of said electrically non-conductive nitrated organic liquid propellant.

2. An improved liquid propellant consisting essentially of a member selected from the group consisting of ethyl nitrate, propyl nitrate, and mixtures thereof, and an additive selected from the group consisting of quaternary ammonium salts and colloidal graphite in an amount of 0.1% to 3.0% by weight.

3. A method for improving the spark ignition of an electrically non-conductive nitrated organic liquid propellant, said method comprising adding to said liquid propellant an additive selected from the group consisting of quaternary ammonium salts and colloidal graphite in an amount effective to permit practical spark ignition of said electrically non-conductive nitrated organic liquid propellant.

10 4. A method for improving the spark ignition of a liquid propellant selected from the group consisting of ethyl nitrate, propyl nitrate, and mixtures thereof, said method comprising adding to said liquid propellant an additive selected from the group consisting of quaternary ammonium salts and colloidal graphite in an amount of 0.1% to 3.0% by weight.

20

#### References Cited

#### UNITED STATES PATENTS

|    |           |         |                 |       |          |
|----|-----------|---------|-----------------|-------|----------|
| 25 | 2,433,943 | 1/1948  | Zwickly et al.  | ----- | 149-89 X |
|    | 2,993,768 | 7/1961  | Holzl           | ----- | 149-89 X |
|    | 3,116,187 | 12/1963 | Scanlon et al.  | ----- | 149-89 X |
|    | 3,148,214 | 9/1964  | Smith           | ----- | 149-88 X |
| 30 | 3,208,891 | 9/1965  | Eschrich et al. | ----- | 149-89 X |

CARL D. QUARFORTH, *Primary Examiner.*

S. J. LECHERT, JR., *Assistant Examiner.*